

## UNITED STATES PATENT OFFICE

2,291,442

## UPPER CYLINDER LUBRICANT

Shaler L. Bass and Eldon F. Graves, Midland,  
Mich., assignors to The Lubri-Zol Corporation,  
Wickliffe, Ohio, a corporation of Ohio

No Drawing. Application November 22, 1938,  
Serial No. 241,810

6 Claims. (Cl. 44—58)

This invention relates, as indicated, to addition agents for internal combustion engine fuels and more particularly to a method of lubricating the upper parts of such engines where extreme conditions of pressure and temperature may obtain. The addition agents of this invention are particularly suited to this purpose by their unusual effectiveness, their stability at high temperatures, and the fact that they are non-corrosive to metals under operating conditions. Further advantages will appear as the description proceeds.

The necessity for adequate lubrication in the upper parts of internal combustion engines has long been apparent and various suggestions have been made for its assurance with equally varying success when carried into practice. When an engine is started there is generally little or no lubricant remaining on the walls of the upper cylinder and excessive wear takes place, especially in cold weather. For this reason top-oilers have been employed by many persons but with not too satisfactory results.

The obvious method of introducing a lubricant to the upper parts of an engine is to employ the fuel as a vehicle and it is one of the objects of this invention to provide an addition agent suited to such purpose.

Another object of this invention is to provide a lubricant capable of resisting the high operating temperatures of internal combustion engines and of affording adequate lubrication to the relatively moving parts under conditions of extreme pressure.

A further object is to provide an addition agent which is unusually effective even when employed in very minor amounts and to provide an engine fuel suitable for consumption by internal combustion engines and which has mixed therewith the addition-agent of this invention.

Still another object of this invention is to provide a lubricating constituent in the fuel acting to lubricate and keep clean the parts of the engine handling the fuel prior to combustion. This problem is particularly acute in Diesel engines where the gumming of orifices and closely fitting parts and the abrasive wear on such parts by the fuel are often excessive.

Thus it will be observed that it is one of the objects of our invention to so modify the fuel used for combustion that it itself will act as a very efficient extreme pressure lubricant prior to the time it is volatilized and consumed by combustion.

Other objects of the invention will appear as the description proceeds.

To the accomplishment of the foregoing and related ends, said invention then consists of the means hereinafter fully described and particularly pointed out in the claims.

The following description sets forth in detail certain approved combinations of ingredients embodying our invention, such disclosed means constituting, however, but certain of various forms in which the principle of the invention may be used.

Broadly stated, this invention comprises a new fuel and method of lubricating the upper parts of internal combustion engines, said fuel comprising the usual liquid hydrocarbons, e. g., gasoline, Diesel fuel, etc., having a viscosity of below 50 sec. Saybolt Universal at 100° F., and a minor amount of an ester of a phosphorus acid, preferably a liquid ester. We have found that of these esters the aromatic esters of phosphoric acid (aromatic phosphates) are the most effective when employed for the purposes of this invention and are therefore preferred.

Of the broad class of aromatic esters of phosphoric acid which may thus be employed in accordance with our invention, the aromatic phosphates containing at least one aromatic radicle having a molecular weight of 100 or more and preferably containing a polyphenyl radicle are generally superior.

The aromatic esters of phosphoric acid, which term is intended to include the alkyl aryl esters, when compounded with the fuel, gasoline, for instance, are found to greatly increase the film strength of the fuel as determined by the well-known Almen machine. The improvement thus obtained makes of the relatively light hydrocarbon employed as fuels and which have very little lubricating value as such, a lubricant with a film strength up to 4 to 5 times that of ordinary good quality untreated lubricating oils. There is apparently a mutual cooperation of the fuel and addition agent to produce a lubricating film of increased film strength inasmuch as the film strength is not only greater than that of either alone but, also, a bearing will operate at lower torque for a given bearing load than with either alone.

The following is a list of particularly effective compounds together with the concentrations in gasoline which afford maximum film strength:

Per cent by weight

|                                      |     |
|--------------------------------------|-----|
| Phenyl di (o-chlor phenyl) phosphate | 0.4 |
| Phenyl di (o-xenyl) phosphate        | 0.5 |
| Di-phenyl mono (o-xenyl) phosphate   | 0.6 |

Since compounds of the type herein disclosed are chemically stable at high temperatures, that is, up to 600-650° F., they are not corrosive to metals under the conditions obtaining in internal combustion engines in operation. Also, the small quantities required are insufficient to necessitate any great correction of the carburetor, etc., nor do they injuriously affect the keeping qualities

of the fuel in storage, often having a contrary effect. The ability to withstand high temperatures without decomposition makes the compounds of this invention particularly adapted for use in Diesel and aviation engines.

If temperatures should ever be reached where these compounds would break down, the resulting phenols and aromatic phosphoric acids would be burned and vented respectively, thus avoiding any deleterious effect upon the metallic parts of the engine.

While larger amounts may be used if desired, the optimum maximum proportion of the addition agent in gasoline is usually on the order of about 0.5% by weight. Depending on the type 15 of fuel and the effect desired, the amount of the addition agent employed may vary from as little as 0.1% to as much as 5.0%.

The word "fuel" as used in this application is intended to include the usual hydrocarbon fuels having a viscosity below 50 sec. Saybolt Universal at 100° F. and a flash point below 200° F. Such fuels will also have distillation points below those of the following table:

10% at 450° F.  
90% at 600° F.  
End at 700° F.

and higher A. P. I. gravity values than 35.

It is thought that the addition agents may 30 chemically or physico-chemically react with the metallic surfaces to form a non-welding surface at points of extreme pressure, thus preventing seizing and scoring with resultant disastrous wear. It is not intended, however, that this invention should be limited by any explanation or theory as to the reasons for the remarkable efficacy of the fuel of this invention.

In summary, the following are among the advantages of this invention:

(1) The upper parts of the engine are effectively lubricated immediately upon the starting of the engine.

(2) Adequate lubrication is afforded at points of extreme pressure despite high temperatures of operation.

(3) Such small quantities of the addition agent are employed that substantially no readjustment of the engine is required.

(4) Friction between relatively moving parts 50 is materially lowered.

(5) A reduction in wear is often noted.

(6) Starting is easier, especially in cold weather.

(7) The fuel is safe to handle, the addition agent being harmless and the exhaust gases having no enhanced deleterious effects.

(8) There is no corrosive effect upon metallic parts.

(9) The fuel is easily prepared.

(10) The fuel injector systems of Diesel engines are kept clean and require fewer repairs.

Other modes of applying the principle of our invention may be employed instead of the one explained, change being made as regards the materials employed, provided the ingredients 5 stated by any of the following claims or the equivalent of such stated ingredients be employed.

We therefore particularly point out and distinctly claim as our invention:

1. As a new composition of matter, an internal combustion engine fuel comprising a liquid hydrocarbon fuel having a viscosity below 50 seconds Saybolt Universal at 100° F., the boiling range of the hydrocarbon content of which has remained substantially unaltered and to which has been added from about 0.1% to about 5.0% by weight, based on the amount of fuel, of a liquid aromatic ester of phosphoric acid containing at least one aromatic radicle having a molecular weight of 100 or more.

2. As a new composition of matter, an internal combustion engine fuel comprising a liquid hydrocarbon fuel having a viscosity below 50 seconds Saybolt Universal at 100° F., the boiling range of the hydrocarbon content of which has remained substantially unaltered and to which has been added from about 0.1% to about 1.0% by weight, based on the amount of fuel, of phenyl di (o-chlor phenyl) phosphate.

3. As a new composition of matter, an internal combustion engine fuel comprising a liquid hydrocarbon fuel having a viscosity below 50 seconds Saybolt Universal at 100° F., the boiling range of the hydrocarbon content of which has remained substantially unaltered and to which has been added from about 0.1% to about 1.0% by weight, based on the amount of fuel, of phenyl di (o-xenyl) phosphate.

4. As a new composition of matter, an internal combustion engine fuel comprising a liquid hydrocarbon fuel having a viscosity below 50 seconds Saybolt Universal at 100° F., the boiling range of the hydrocarbon content of which has remained substantially unaltered and to which has been added from about 0.1% to about 1.0% by weight, based on the amount of fuel, of di-phenyl mono (o-xenyl) phosphate.

5. An internal combustion engine fuel the boiling range of the hydrocarbon content of which has remained substantially unaltered and to which has been added from about 0.1% to about 5.0% of an aromatic ester of phosphoric acid containing a poly-phenyl radicle.

6. An internal combustion engine fuel comprising from about 99.9% of the usual hydrocarbon fuel and 0.1% of an ester of an acid of phosphorus to about 95% of such fuel and 5% of an ester of an acid of phosphorus.

SHAILER L. BASS.  
ELDON F. GRAVES.